

## UNITED STATES PATENT OFFICE.

ARMAN E. BECKER, OF ELIZABETH, NEW JERSEY, ASSIGNOR TO STANDARD DEVELOPMENT COMPANY, A CORPORATION OF DELAWARE.

## METHOD OF LUBRICATING INTERNAL-COMBUSTION ENGINES.

No Drawing.

Application filed October 29, 1925. Serial No. 65,697.

This invention relates to an improved method of lubricating internal-combustion engines. In accordance with the invention, the crank-case of the engine is supplied with 5 a hydrocarbon lubricant containing a small percentage of a saponified compound, especially an alkali metal soap of a high fatty acid or acids. The oil-soap lubricant, in a preferred 10 form, comprises lubricating oil of good grade containing a sodium soap in effective amount less than 0.5% by weight of the oil. However, my invention is not limited to precise proportions of soap and oil, and any 15 composition having the desired viscosity and lubricating qualities at engine temperature may be used. In general more than 0.5% of soap will cause the formation of a gel at ordinary temperatures with oils of viscosity 20 high enough for best results in internal-combustion engines. In cases where light lubricating oils are satisfactory, higher percentages of soap may be used without solidification. Lubricating oil of about 285 to 290 25 seconds Saybolt viscosity at 100° F. containing about 0.15 to 0.25% of a sodium soap, especially sodium oleate, gives excellent results. An intermediate percentage, say 0.17%, has given a maximum benefit on extensive tests.

It will be clear as the description proceeds, that the effect of the soap is not merely to increase the viscosity of the lubricating oil nor merely to improve its lubricating properties. In all cases I prefer to use an oil having in itself characteristics adapting it for advantageous use as an internal-combustion engine cylinder oil. My invention is based upon the discovery that the soap has 35 special functions, especially in connection with parts liable to fouling by carbonaceous or gummy deposits. An incidental feature of my invention is the effect of the soap in reducing friction on bearings and all moving parts, and in permitting the desirable "fluid film" lubrication over a wider range of speeds and loads for a given feed of oil.

In some cases I use a white oil or other 40 highly purified hydrocarbon oil of lubricating characteristics and containing a soap of the type described. Such oils resist oxidation and other chemical changes much better than the cheaper lubricating oils of ordinary type, and the use of white oils is there-

fore justified by their increased length of 55 service. The percentage of soap compounded with white oils or the like may be the same as above mentioned.

In preparing the oil-soap lubricant it is generally desirable to apply heat. This facilitates solution and obviates the tendency of the soap to separate from the oil, a difficulty which may be encountered in solutions prepared by mixture at ordinary temperature. The process of forming the oil-soap lubricant forms no part of the present invention, but is included in the subject matter of my pending United States patent applications Serial Nos. 593,906, filed October 11, 1922, and 751,401, filed November 21, 70 1924.

I have found by extensive tests under laboratory and service conditions that the presence of a soap of the type described in an internal-combustion engine lubricant 75 has a marked beneficial effect. The tendency to carbon formation upon the cylinder walls is greatly reduced and detonation or "knocking" in the engine is minimized. In many cases removal of carbon already formed has 80 been effected by the use of my lubricating composition. Among other advantages, a reduction of engine temperature and increased horse-power result from the practice of this invention.

The water which may be formed by condensation in the crank-case has no adverse effect upon the oil-soap lubricant. In fact, in many cases small amounts of water, say 85 up to 2 or 3%, appear to increase somewhat 90 the efficiency of the lubricant.

A further important advantage of the oil-soap composition is its action on the transmission and brake bands of motor vehicles having a planetary gear transmission. The 95 fouling with carbon or glazing of the surface of the bands is substantially prevented and the resulting objectionable "chattering" is minimized. In those cars having the planetary mechanism and bands in a case 100 opening into the crank-case, the oil-soap lubricant supplied to the crank-case will serve for treating the bands. The action on the bands may be in part a softening or deglazing effect, but I shall refer to it generally 105 herein as lubrication.

My invention is applicable to the lubrication of internal-combustion engines of all

types, including Diesel engines. The specific details given as to the lubricant to be used are illustrative of preferred procedure only, and various modifications may be made 5 within the scope of the appended claims, in which it is my intention to claim all novelty inherent in the invention as broadly as the prior art permits.

I claim:

- 10 1. Method of lubricating internal-combustion engines and associated parts, comprising supplying to surfaces tending to become fouled with carbonaceous or gummy deposits, a liquid composition consisting essentially of lubricating oil containing an alkali metal soap of a fatty acid in an effective amount less than 0.5% by weight of the oil.
- 15 2. Method of lubricating internal-combustion engines, comprising supplying to the cylinder walls of the engine a liquid composition consisting essentially of lubricating oil containing an alkali metal soap of a high fatty acid in an effective amount less than 0.5% by weight of the oil.
- 20 3. Method of lubricating internal-combustion engines, comprising maintaining in the crank-case of the engine a quantity of a liquid composition consisting essentially of lubricating oil containing an alkali metal
- 25 soap of a high fatty acid in an effective amount less than 0.5% by weight of the oil,

and supplying the same to the cylinder walls of the engine.

4. Method of lubricating internal-combustion engines, comprising maintaining in the 35 crank-case of the engine a quantity of a liquid composition consisting essentially of lubricating oil containing about 0.15 to 0.25% by weight of a sodium oleate, and supplying said oil-soap lubricant to the cylinder 40 walls of the engine.

5. Method of lubricating internal-combustion engines, comprising maintaining in the crank-case of the engine a quantity of a liquid composition consisting essentially of 45 highly purified lubricating oil of the type of white oil and containing a soap in effective amount less than 0.5% by weight of the oil, and supplying said oil-soap composition to the cylinder walls of the engine. 50

6. Method of lubricating internal-combustion engines, comprising maintaining in the crank-case of the engine a quantity of a liquid composition consisting essentially of highly purified lubricating oil of the type 55 of white oil and containing a sodium soap of a high fatty acid in an effective amount less than 0.5% by weight of the oil, and supplying said oil-soap composition to the cylinder walls of the engine.

ARMAN E. BECKER.